

## UNITED STATES PATENT OFFICE

2,216,535

## STAINLESS STEEL

James R. Long, Annapolis, Md., assignor to Chicago Development Company, Chicago, Ill., a corporation of Illinois

No Drawing. Application April 2, 1938,  
Serial No. 199,602

2 Claims. (Cl. 75—128)

My invention relates to stainless steels, particularly stainless steels employing manganese, and used in the austenitic state. Commercial stainless steels, in general, comprise iron, nickel and chromium. The type of stainless steel finding the greatest commercial applications is the so-called 18-8 steel which consists of 18% chromium, 8% nickel and the remainder iron. This steel is truly austenitic, capable of being handled and worked in the cold state and having very great advantages in the fabrication of stainless steel machinery parts, retorts, chemical reaction vessels and the like. The stainless steel of the cutlery type is, in general, not austenitic and my invention is not primarily concerned with this particular type of product.

Because of the scarcity and the relatively high cost of nickel and for other reasons, the replacement of nickel by some other metal has received special consideration, particularly in such countries as Germany. Manganese has been considered as a substitute for nickel and it has been found that manganese is only partially effective in changing the body centered ferrite of chromium iron into face centered austenite. In such steels as have been produced employing manganese, it has been necessary to raise the carbon content and also to use an appreciably greater proportion of manganese to obtain the austenitic stainless steel properties found in 18-8 steel.

The relation between the carbon content and manganese necessary to produce a completely austenitic alloy is clear from the work of Bain, Davenport and Waring. The results obtained by these investigators are not fully conclusive because their work extended only up to 14% manganese at which percentage approximately 0.2% of carbon was found to be required to produce a completely austenitic alloy. By extrapolation it would appear from this work that approximately 20% of manganese would produce a completely austenitic alloy, but further work reported in "The Metallurgist" of February 26, 1937, shows that with 15% manganese and 20% of chromium 0.3% of carbon must be employed to give the desirable austenitic character to the alloy.

The increase of the carbon content in alloys of the type discussed has certain disadvantages. In such alloys as 18% chromium and 10% manganese with sufficient carbon to insure completely austenitic properties, a hard brittle constituent is precipitated which has been tentatively identified as the B constituent of Bain and Griffith. This compound is an iron-chromium

compound, the stability of which is definitely questioned in pure alloys. Heycock reported an inability to find this compound in pure alloys. The use of increased carbon is also objectionable because increased carbon tends to cause susceptibility to inter-granular corrosion. Inhibitors such as columbium and titanium can not be used to inhibit such inter-granular corrosion, because such metals employed as inhibitors would completely extract the carbon from the manganese carbide.

The best outlook for the satisfactory production of high manganese austenitic stainless steels, in view of this situation, would, therefore, appear to be through a considerable increase in the manganese content. Proceeding in this direction, however, has shown the tendency to produce the so-called epsilon phase which occurs in iron-manganese alloys containing 12 to 20% of manganese and very low carbon. The conditions for the stability of this epsilon phase as well as the conditions for the stability of the B phase of the iron-chromium system have not been definitely determined. Nevertheless, the very distinct presence of the two phases under conditions found in the past has necessarily resulted in investigators proceeding in a somewhat different direction to produce true austenitic stainless steels of good grade.

Because of this situation, some attention has been directed towards the production of stainless steels which are only in part austenitic. It has been found that an alloy of 18% chromium, 8% manganese, 1% copper and 0.1% carbon when rapidly cooled from 1925 degrees F. will produce a structure which is approximately 60% austenite and 40% ferrite. Steels of this kind have received some attention and for some purposes have been considered to show some promise. Kinzel has stated that these duplex steels have a definite place in the industry since they are easier to cold work and machine than the austenitic alloys. Their cold drawing properties, however, are definitely inferior. An alloy of 18% chromium, 6% manganese, 4% nickel and 1% of copper has been found to be austenitic and is substantially equal to 18-8 steels in corrosion resistance and working properties.

One object of my invention is the provision of an improved austenitic stainless steel having as a constituent thereof a substantial quantity of manganese.

Another object is the utilization of manganese and nickel in such a manner as to assure austenitic properties with either no carbon or such

a small amount of carbon as to have little or no deleterious effect on the steel such as identified hereinbefore.

Another object is the improved use of manganese in stainless steels.

In the development of my invention I found that so-called pure manganese as it was delivered commercially to experimenters in general contained as much as 6% of impurities, generally iron, silicon, carbon, sulphur and aluminum. The iron content of manganese is not of primary significance when working on stainless steels, but the presence of significant quantities of silicon and aluminum, above 1 and  $\frac{1}{2}$ % of the manganese, I considered possibly to be of significant interest. I proceeded on the assumption that the silicon and aluminum content of manganese had to a considerable extent been overlooked by investigators and that this might account to a substantial extent for the results obtained. To this end I was led to a consideration of substantially pure manganese produced by the distillation of commercially pure manganese in vacuum or by the electrolysis of pure manganese sulphate solutions. Methods for producing substantially pure manganese have been given in the literature and need not be repeated here. I find that by the use of high purity manganese, desirable results are obtained in the use of large proportions of manganese for the production of stainless steels, very little, if any, carbon being required to keep the alloy in the austenitic state. I, therefore, accomplish the objects of my invention primarily by the use of a high purity manganese so that the final alloy will have a minimum carbon content and contain a minimum amount of impurities as silicon and aluminum, all as will be more fully described hereinafter.

For the convenience of those skilled in the art I shall refer more in particular to the character of the manganese employed.

For the purpose of comparison, I give below the analyses of two samples of commercial manganese:

|           | Per cent |
|-----------|----------|
| No. 1:    |          |
| Manganese | 96.74    |
| Silicon   | 0.76     |
| Carbon    | 0.03     |
| Sulphur   | 0.09     |
| Aluminum  | 0.88     |
| No. 2:    |          |
| Manganese | 94.71    |
| Silicon   | 1.56     |
| Carbon    | 0.18     |
| Aluminum  | Trace    |

By purifying commercial manganese by either of the methods set out hereinabove, I have been able to produce a manganese product containing less than 0.1% of any of the elements iron, carbon, silicon and aluminum and wherein the sum of these elements present in the manganese is less than 0.3%. A manganese of this type, I have found, possesses entirely different properties in stainless steels than the manganese heretofore utilized in metallurgical work and presumably considered adequately pure for alloying purposes. The impurities present in the manganese, particularly silicon and aluminum, if present in appreciable quantities seem to be exceedingly powerful in preventing retention of the austenite. It is significant that the stainless steel described in the article in "The Metallurgist" referred to

hereinaabove and which requires 0.3% of carbon to retain the desirable austenitic state analyzed 0.54 to 0.79% silicon. Unquestionably the presence of this relatively large proportion of silicon, introduced probably through the use of a commercial source of manganese, accounted in part for the fact that 0.3% of carbon was required in this particular alloy.

I found that the following range of proportions may be employed to produce substantially the properties of 18-8 stainless steel, modified slightly, to be sure, when the extreme of the range indicated is employed: nickel 0 to 5%, manganese 10 to 30% or more, chromium 10 to 20%, and the remainder iron. The manganese which I employ in all instances contains less than 0.3% iron, carbon, aluminum and silicon and less than 0.1% of any one of these substances.

A small proportion of carbon may be present in the alloys of my invention without deleteriously affecting them. Indeed, up to 0.15% carbon may under certain circumstances be advantageous. At no time, however, do I have present more than 0.15% of carbon in the alloy as a whole.

The silicon and aluminum must be very carefully controlled in order to produce satisfactory results with my invention because these two substances, normally found in commercial manganese, tend to prevent the production of an austenitic alloy. While it is possible that some silicon and aluminum may be introduced through the iron or chromium, in general, the production of these two materials has been so controlled in the past that substantially silicon and aluminum free materials may be obtained. However, in so far as there may be silicon or aluminum present, the proportion of these two impurities so found must be taken into consideration. In general, however, if the manganese is highly purified so as to contain less than 3% of the compounds iron, carbon, silicon and aluminum, very satisfactory results can be obtained by the practice of my invention. In general, the total of aluminum and silicon should not be more than 0.15% based upon the weight of the manganese present, and dependable results can be obtained if this figure be not exceeded.

The stainless steel produced in accordance with my invention is obtained entirely in the austenitic stage by ordinary cooling. This stainless steel or stainless iron can be produced by, in general, substituting for all or a part of the nickel heretofore employed in stainless steel an equal or greater proportion of manganese purified to such a state that the sum of iron, carbon, silicon and aluminum present in the manganese is less than 0.3%. It is not to be assumed that my invention is limited to the presence of 15% of manganese as referred to in the specific example given hereinabove. I may employ 30% or more of substantially chemically pure manganese such as that described and produce steels having excellent properties. While I have not been able to determine all of the properties of such steels, I have found that the so-called epsilon phase very often found in high manganese content alloys is avoided and also conditions do not seem to favor the stability of the B constituent referred to hereinabove. Furthermore, apparently because of the absence of impurities, other disadvantages heretofore found when the manganese was increased appreciably, do not seem to occur. When very high manganese is employed I have not deter-

mined fully whether or not the resulting alloy is entirely austenitic under all conditions of time and temperature employed in treatment, but it appears that the alloys are either substantially 5 entirely austenitic or contain such appreciable quantities of the austenitic phase that they have excellent working properties and from a tensile strength and hardness standpoint they are suitable for many uses where stainless steel is customarily used.

10 It should be kept in mind that my invention is capable of considerable variation while still producing alloys having the general properties found desirable in stainless chromium steels. For example, an alloy of manganese 30%, chromium 18%, nickel 2% and balance iron is entirely austenitic and has very excellent properties making it very suitable for use in the industries where high corrosion resistance and strength are desired. In a true type of stainless iron the nickel may, as suggested, be replaced entirely by the manganese with good results, the proportion of manganese being increased with increase of chromium and reduction of nickel so that in the 15 higher chromium substantially nickel free alloys, more than 30% manganese may be required to secure the desired properties described.

20 While the stainless steels of my invention do not require the presence of copper or other materials heretofore employed in certain modified

stainless steels, I may, if desired, add minor proportions of other constituents such as copper while still maintaining the balance of silicon, aluminum and carbon described.

What I claim as new and desire to protect by Letters Patent of the United States is:

1. An austenitic stainless steel alloy of iron, chromium, nickel and manganese, said alloy as a whole having less than 0.15% carbon and less than 0.15% total of silicon and aluminum based 10 upon the manganese content, said alloy consisting of manganese, 10 to 30%; substantially pure chromium, 10 to 20%; nickel, .5% to 5%; balance, substantially pure iron; said manganese being of a highly pure grade and containing not 15 more than about .1% by weight of any one of the elements carbon, silicon and aluminum.

2. An austenitic stainless steel comprising nickel up to about 5%, manganese from 10 to 15%, chromium from 16 to 20% and the remainder iron, said alloy as a whole having less than 0.15% carbon, and the total content of silicon and aluminum being less than 0.15% based 20 upon the manganese present, each of said elements nickel, chromium and iron being substantially pure, and said manganese being highly purified and containing not more than .1% of any one of the elements carbon, silicon and aluminum. 25

JAMES R. LONG. 30